# EUROPEAN PATENT SPECIFICATION

(11) **EP 0 220 964 B1**
(45) Date of publication and mention of the grant of the patent: **18.09.1991**
(21) Application number: 86308445.5
(22) Date of filing: 29.10.1986
(51) Int. Cl.: B24D 3/00

(54) **Cubic boron nitride abrasive bodies**
Schleifkörper aus kubischem Bornitrid
Outil abrasif en nitrure de bore cubique

(30) Priority: 30.10.1985 ZA 858339
(43) Date of publication of application: 06.05.1987
(73) Proprietor: DE BEERS INDUSTRIAL DIAMOND DIVISION (PROPRIETARY) LIMITED, Johannesburg Transvaal (ZA)
(72) Inventor: Phaal, Cornelius, Craighall Park Johannesburg Transvaal (ZA); Dodsworth, John, Constantia Kloof, Florida§Transvaal (ZA)
(74) Representative: Jones, Alan John

(56) References cited:
- EP-A- 0 101 259
- FR-A- 2 285 213
- US-A- 3 743 489
- US-A- 3 944 398
- US-A- 4 401 443
- CHEMICAL ABSTRACTS, vol. 104, no. 20, 19th May 1986, page 269, abstract no. 172825e, Columbus, Ohio, US; & JP-A-60 263 602 (SUMITOMO ELECTRIC INDUSTRIES, LTD) 27-12-85
- Idem

## Description

### BACKGROUND OF THE INVENTION

This invention relates to cubic boron nitride abrasive bodies.

Cubic boron nitride abrasive compacts are known in the art (e.g. EP-A1-0 101 259) and consist of a polycrystalline mass of cubic boron nitride particles present in an amount of at least 70 percent by volume bonded into a hard conglomerate. Such compacts may contain a second phase. When provided, the second phase is typically a ceramic phase. The second phase acts to some extent as a binder phase for the cubic boron nitride particles.

One of the most successful cubic boron nitride abrasive compacts presently on the market is one wherein the second phase consists essentially of aluminium nitride and/or aluminium diboride. This compact is sold in the form of large discs which are clamped into a suitable tool holder and used in this manner for abrading various work pieces. A curved edge of the compact is used as the abrading edge. This compact is designed for applications where a high removal rate of workpiece is desired.

Abrasive compacts comprising diamond or cBN abrasive particles or a mixture thereof, present in an amount of at least 50 volume percent, bonded into a hard conglomerate by means of a metal are known from US-A-4 063 909. According to this document the compacts are bonded to a support by a layer of high temperature braze with a thickness of less than 0.5 mm. Suitable high temperature braze metals include Ti, Ni, Co, Fe, Cr, Mn, V, Mo, Ta or Pt or an alloy containing one or more thereof, Ti or Ti-alloys are particularly preferred.

### SUMMARY OF THE INVENTION

According to the present invention, there is provided a tool insert comprising an abrasive compact comprising a polycrystalline mass of cubic boron nitride particles present in an amount of at least 70 percent by volume and containing substantial direct particle-to-particle bonding and a second phase dispersed through the cubic boron nitride particle mass, the abrasive compact presenting major surfaces on each of opposite sides thereof, the one major surface providing a cutting point for the insert and the other major surface having bonded thereto, and being in direct contact with, a layer of molybdenum of thickness less than 0,5mm, the largest linear dimension of the compact being no more than 10mm.

### DETAILED DESCRIPTION OF THE INVENTION

The tool insert of the invention is thus a small cubic boron nitride compact which has a molybdenum layer bonded to one major flat surface thereof. Because of its size, it is not practical to hold the insert mechanically in a suitable tool holder. However, the presence of the molybdenum layer renders the compact brazeable to a tool holder. It is preferable that the compact is first brazed to a cemented carbide support which is then brazed to the tool holder or mechanically held in a tool holder. Cemented carbide has a similar coefficient of thermal expansion to the compact and problems arising due to differences in thermal expansion of the compact and support are minimised.

The abrasive compact of the insert preferably has a rectangular, triangular, pentagonal or hexagonal shape. Thus, the compact presents several points and it is these points which provide cutting points for the insert.

The molybdenum layer is the thin layer, preferably having a thickness in the range 50 to 150µm (microns). The layer of molybdenum may have an outer nickel or like metal layer applied to it, that is to say, the layer of molybdenum is in direct contact with the abrasive compact and is between the abrasive compact and the nickel or like metal layer. The cubic boron nitride compact may be any known in the art but is preferably one wherein the second phase contains aluminium nitride and/or aluminium diboride. Second phases of this nature are produced when aluminium is present during manufacture of the compact. One particularly preferred cubic boron nitride of this nature has a second phase which consists essentially of aluminium nitride and/or aluminium diboride. The second phase may also contain other components such as silicon which is either in elemental or combined form.

The tool inserts of the invention may be used for a wide variety of applications. They have particular application for light to medium turning, boring, grooving, threading and milling of various steels, irons and alloys such as:
Ni-HARD white irons having a hardness of 55 to 58 HRC
High chromium irons having a hardness of 55 to 62 HRC
Cold work tool steels having a hardness of 60 HRC
High speed steels having a hardness of 62 HRC
Grey cast irons (pearlitic) having a hardness of 220 HB
Sintered irons having a hardness of 100 HB
Cobalt-based hard facing alloys
Nickel-based hard facing alloys
Meehanite white irons having a hardness of 55 HRC

In all these applications the cubic boron nitride abrasive compact will be brazed to a cemented carbide support, preferably a cemented tungsten carbide support, by means of the readily brazeable molybdenum layer and using a braze such as a silver brazing alloy having a melting point between 660°C and 840°C. The thus bonded cubic boron nitride abrasive compact will then be held mechanically or brazed to the shank of a tool and used in this form for the various abrading applications mentioned above.

As mentioned above, the tool insert is particularly useful for light to medium cut applications. This means that the infeed of the tool insert during turning, boring, grooving or milling will not exceed 0,3mm per revolution or pass of the insert across the workpiece.

In an example of the invention, a mass of cubic boron nitride particles was placed in contact with an aluminium foil which itself was placed in contact with a foil of molybdenum. This unbonded assembly was placed in the reaction zone of a conventional high temperature/high pressure apparatus and subjected to a temperature of about 1500°C and a pressure of about 5.5Gpa (55 kilobars) for a period of 15 minutes. Recovered from the reaction zone using conventional techniques was an abrasive compact containing about 90 percent by volume of cubic boron nitride particles in which there was substantial direct particle-to-particle bonding and a second phase consisting essentially of aluminium nitride and/or aluminium diboride. The compact was produced in the form of a disc and had bonded to a major flat surface thereof a layer of molybdenum of thickness about 100µm (microns). This compact was cut into a plurality of equilateral triangles, some having a side dimension of 5mm and others having a side dimension of 7mm. Each triangle constituted a tool insert of the invention.

The triangular-shaped inserts produced in this manner were found to be excellent for the boring of pearlitic grey cast iron, for the facing of Stellite 6 hard facing alloy and the threading of Ni-HARD white cast iron. The particular conditions used in each example are given below.

| EXAMPLE 1 - BORING | |
|---|---|
| Material | Pearlitic grey cast iron |
| Hardness | 220 HB |
| Speed | 600m/min |
| Feed | 0,2mm/rev |
| Cut | 0,5mm |
| Coolant | None |

| EXAMPLE 2 - FACING | |
|---|---|
| Material | Stellite 6 hard facing alloy |
| Hardness | 30 HRC |
| Speed | 200m/min |
| Feed | 0,2mm/rev |
| Cut | 0,5mm |
| Coolant | None |

| EXAMPLE 3 - THREADING | |
|---|---|
| Material | Ni-HARD white cast iron |
| Hardness | 58 HRC |
| Speed | 40m/min |
| Thread form | ISO M16 |
| Radial infeed | 0,1mm/pass |
| Coolant | None |

## Claims

1. A tool insert comprising an abrasive compact comprising a polycrystalline mass of cubic boron nitride particles present in an amount of at least 70 percent by volume and containing substantial direct particle-to-particle bonding and a second phase dispersed through the cubic boron nitride particle mass, the abrasive compact presenting major surfaces on each of opposite sides thereof, the one major surface providing a cutting point for the insert and the other major surface having bonded thereto, and being in direct contact with, a layer of molybdenum of thickness less than 0,5mm, the largest linear dimension of the compact being no more than 10mm.

2. A tool insert according to claim 1 wherein the second phase contains aluminium nitride and/or aluminium diboride.

3. A tool insert according to claim 1 or claim 2 wherein the second phase contains silicon in elemental or combined form.

4. A tool insert according to any one of the preceding claims wherein the thickness of the molybdenum layer is in the range of 50 to 150µm (microns).

5. A tool insert according to any one of the preceding claims wherein the compact has a triangular, rectangular, pentagonal or hexagonal shape .

6. A tool insert according to any one of the preceding claims wherein the cubic boron nitride compact is brazed to a cemented carbide support by means of the molybdenum layer and a braze.

7. A tool insert according to claim 6 wherein the braze is a silver brazing alloy having a melting point between 660°C and 840°C.

8. A method of abrading a workpiece in a light to medium cut application, i.e. wherein the infeed of the tool insert does not exceed 0.3 mm per revolution or pass of the insert across the workpiece, including the step of causing the workpiece to be contacted in an abrading manner by the cutting point of a tool insert according to any one of claims 1 to 7.

9. Use of a tool insert according to any one of claims 1 to 7 in a light to medium cut application, i.e. wherein the infeed of the tool insert does not exceed 0.3 mm per revolution or pass of the insert across the workpiece.

10. A tool comprising the tool insert of any one of claims 1 to 7.

## Revendications

1. Insert d'outil comprenant un corps compact abrasif constitué par une masse polycristalline de particules de nitrure de bore cubique présentes dans une quantité d'au moins 70 % en volume et contenant une liaison importante directe de particule à particule et une seconde phase dispersée dans la masse de particules de nitrure de bore cubique, le corps compact abrasif présentant des surfaces principales sur chacun de ses côtés opposés, la surface principale fournissant un point de coupe pour l'insert et l'autre surface principale comportant une couche de molybdène d'une épaisseur inférieure à 0,5 mm liée sur celle-ci, et étant en contact direct, la plus grande dimension linéaire du corps compact n'étant pas supérieure à 10mm.

2. Insert d'outil selon la revendication 1, dans lequel la seconde phase contient du nitrure d'aluminium et/ou du diborure d'aluminium.

3. Insert d'outil selon la revendication 1 ou 2, dans lequel la seconde phase contient du silicium sous la forme élémentaire ou combinée.

4. Insert d'outil selon l'une quelconque des revendications précédentes dans lequel l'épaisseur de molybdène se situe dans la plage de 50 à 150 microns.

5. Insert d'outil selon l'une quelconque des revendications précédentes dans lequel le corps compact présente une forme triangulaire, rectangulaire, pentagonale ou hexagonale.

6. Insert d'outil selon l'une quelconque des revendications précédentes dans lequel le corps compact en nitrure de bore cubique est brasé sur un support en carbure cémenté au moyen de la couche de molybdène et d'une brasure.

7. Insert d'outil selon la revendication 6, dans lequel la brasure est un alliage de brasure en argent ayant un point de fusion situé entre 660°C et 840°C.

8. Procédé pour l'abrasion d'une pièce à usiner dans une application de coupe légère à moyenne, c'est-à-dire dans lequel l'avance de l'insert d'outil ne dépasse 0,3 mm par tour ou passe de l'insert sur la pièce à usiner, comprenant l'étape consistant à mettre la pièce à usiner en contact d'une manière abrasive par le point de coupe d'un insert d'outil selon l'une quelconque des revendications 1 à 7.

9. Utilisation d'un insert d'outil selon l'une quelconque des revendications 1 à 7 dans une application de coupe légère à moyenne, c'est-à-dire dans laquelle l'avance de l'insert de l'outil ne dépasse pas 0,3 mm par tour ou passe de l'insert sur la pièce à usiner.

10. Outil comprenant l'insert d'outil selon l'une quelconque des revendications 1 à 7.

## Patentansprüche

1. Werkzeugeinsatz, umfassend einen Schleifcompact, der eine polykristalline Masse von kubischen Bornitrid-Teilchen umfaßt, die in einer Menge von wenigstens 70 Vol.-% vorhanden sind und in erheblichem Maße direkte Teilchen-zu-Teilchen-Bindung enthält, und eine durch die Masse aus kubischen Bornitrid-Teilchen dispergierte zweite Phase, wobei der Schleifcompact an jeder seiner gegenüberliegenden Seiten Hauptflächen aufweist, wobei die eine Hauptfläche eine Schneidkante für den Einsatz liefert, und die andere Hauptfläche eine Molybdän-Schicht mit einer Dicke von weniger als 0,5 mm an sich gebunden hat und damit in direktem Kontakt ist, wobei die größte lineare Ausdehnung des Compacts nicht größer als 10 mm ist.

2. Werkzeugeinsatz nach Anspruch 1, wobei die zweite Phase Aluminiumnitrid und/oder Aluminiumdiborid enthält.

3. Werkzeugeinsatz nach Anspruch 1 oder 2, wobei die zweite Phase Silicium in elementarer oder kombinierter Form enthält.

4. Werkzeugeinsatz nach irgendeinem der vorstehenden Ansprüche, wobei die Dicke der Molybdän-Schicht im Bereich von 50 bis 150 µm (Mikron) liegt.

5. Werkzeugeinsatz nach irgendeinem der vorstehenden Ansprüche, wobei der Compact eine dreieckige, rechteckige, pentagonale oder hexagonale Form hat.

6. Werkzeugeinsatz nach irgendeinem der vorstehenden Ansprüche, wobei der Compact aus kubischem Bornitrid vermittels der Molybdän-Schicht und einem Lot auf einen Sintercarbid-Träger gelötet ist.

7. Werkzeugeinsatz nach Anspruch 6, wobei das Lot eine Silber-Lötlegierung ist, die einen Schmelzpunkt zwischen 660°C und 840°C hat.

8. Verfahren zum Schleifen eines Werkstücks bei leichten bis mittleren Schneideverwendungen, d.h., wobei der Vortrieb des Werkzeugeinsatzes 0,3 mm pro Umdrehung oder Schnitt des Einsatzes über das Werkstück nicht übersteigt, umfassend die Stufe, bei der das Werkstück mittels der Schleifkante eines Werkzeugeinsatzes gemäß irgendeinem der Ansprüche 1 bis 7 in einer schleifenden Weise in Kontakt gebracht wird.

9. Verwendung eines Werkzeugeinsatzes nach irgendeinem der Ansprüche 1 bis 7 bei leichten bis mittleren Schneideververwendungen, d.h., wobei der Vortrieb des Werkzeugeinsatzes 0,3 mm pro Umdrehung oder Schnitt des Einsatzes über das Werkstück nicht übersteigt.

10. Werkzeug, umfassend den Werkzeugeinsatz nach irgendeinem der Ansprüche 1 bis 7.
